

**1**

2,885,363

**EXTREME PRESSURE LUBRICANT**

George Wolfram and Joseph B. Stucker, Des Plaines, Ill., assignors to The Pure Oil Company, Chicago, Ill., a corporation of Ohio

No Drawing. Application October 20, 1953  
Serial No. 387,324

2 Claims. (Cl. 252—46.6)

This invention relates to lubricants and methods of preparing the same, and more particularly to lubricant additives which impart extreme pressure characteristics to lubricants and methods for the preparation thereof.

It has long been known in the art of lubrication that the addition of sulfurized or sulfurized and phosphorized fatty material to lubricants will greatly increase the extreme pressure characteristics of the lubricant. For example, sulfurized fatty materials, such as lard oil and the like, have heretofore been used to increase the extreme pressure properties of mineral oil base and emulsion type metal working lubricants, such as cutting oils, and other lubricants which are subjected to high pressure during use. Likewise, sulfurized and phosphorized fatty materials have been used to increase the extreme pressure properties of lubricants, particularly automotive gear lubricants. Examples of the latter type of lubricants and their methods of preparation may be found in United States Patents 2,211,231 to Lawrence M. Henderson, issued August 13, 1940, and 2,211,306 to William A. Whittier et al., issued August 13, 1940. Although lubricants prepared and blended in accordance with the above and other patents relating to lubricants containing sulfurized or sulfurized and phosphorized fatty materials have satisfactory extreme pressure characteristics, they have been found deficient in certain other characteristics. One notable deficiency of the sulfurized or sulfurized-phosphorized fatty materials of the prior art has been their lack of universal solubility in mineral lubricating oils. This lack of compatibility with mineral oils has been particularly vexing when attempts are made to incorporate extreme pressure additives in high viscosity index mineral oils such as Pennsylvania and Mid-Continent solvent refined oils. Inasmuch as extreme pressure additives of the type referred to above lack compatibility in high viscosity index oils, another serious drawback in the preparation of extreme pressure lubricants is the inability to obtain lubricants possessing both extreme pressure characteristics and high viscosity index characteristics. Difficulties have also been experienced in the preparation of extreme pressure lubricants of satisfactory low temperature characteristics. This problem is evidenced by the fact that the lubricants fail to remain fluid at low temperatures and thus do not provide proper lubrication at winter temperatures in temperate geographical zones.

It is, therefore, an object of the present invention to provide improved extreme pressure additives and lubricant blends containing these additives.

Another object of this invention is to provide extreme

**2**

pressure lubricant additives having improved solubility in mineral oil lubricants.

Another and further object of this invention is to provide extreme pressure lubricants having improved viscosity index characteristics.

Still another object of this invention is to provide extreme pressure lubricants having improved low temperature characteristics.

A further object of this invention is to provide extreme pressure lubricants having improved viscosity index characteristics and improved low temperature characteristics.

A still further object of this invention is to provide sulfurized and sulfurized-phosphorized lubricant additives having improved solubility in high viscosity index mineral oils.

Still another object of this invention is to provide improved methods of preparing extreme pressure lubricant additives having improved solubility in mineral oil lubricants and extreme pressure lubricants having improved viscosity index and low temperature characteristics.

Other and further objects of this invention will be apparent from the following detailed description of the invention.

In accordance with the present invention, it has been found that the presence of fatty esters containing polyethenoid linkages (also referred to as polyunsaturated glycerides) in fatty materials which are sulfurized or sulfurized and phosphorized to form extreme pressure lubricant additives adversely affects the solubility of such additives in mineral oils and the viscosity index characteristics of lubricants prepared therefrom. Although it is not intended to limit the scope of the invention by a theoretical explanation, it is believed that the polyunsaturated glycerides enter into a chemical reaction either by polymerization or by combining with sulfur or sulfur and phosphorous to form oil-insoluble materials during the preparation of extreme pressure lubricant additives by sulfurization or sulfuration and phosphorization. Thus, it has been found that extreme pressure lubricant additives which are universally soluble in mineral oils and which form lubricants of improved viscosity index characteristics when blended with mineral oils can be prepared by counteracting the effect of the polyunsaturated glyceride content of the fatty materials used in the preparation of sulfurized or sulfurized and phosphorized extreme pressure lubricant additives. The term "counteract" as used herein is meant to include reducing the polyunsaturated glyceride content of fatty materials prior to sulfurization or sulfuration and phosphorization as well as neutralizing or rendering inactive the polyunsaturated glycerides of fatty materials having normal polyunsaturated glyceride content. It has also been discovered in accordance with the present invention that the low temperature characteristics of lubricants prepared from sulfurized or sulfurized and phosphorized fatty materials whose polyunsaturated glyceride content has been rendered inactive can be improved by counteracting the effect of the high melting point saturated fatty acid esters and, more particularly, the glyceryl esters of stearic, palmitic and myristic acids present in the fatty material. By thus reducing or rendering inactive the glyceryl esters of stearic, palmitic and myristic acids, the low temperature

characteristics of the lubricants of this invention can be improved without adversely affecting the solubility and viscosity index characteristics of the lubricant.

Extreme pressure lubricant bases prepared according to the methods of sulfurizing and phosphorizing fatty oils described in United States Patents 2,211,231 and 2,211,306, supra, have been found to have limited solubility in lubricating mineral oils. Such extreme pressure lubricant bases are compatible with only limited types of mineral oil such as Gulf Coastal lubricating mineral oils and Mid-Continent conventionally refined lubricating mineral oils when the Mid-Continent conventionally refined oil is kept at a minimum. However, the extreme pressure lubricant bases prepared according to the methods described in the above-mentioned United States patents have poor compatibility with high viscosity index

5 cent. The second extreme pressure lubricant base was prepared using lard oil of low polyunsaturated glyceride content (hereinafter referred to as LPU lard oil) in the range of 1 to 2 percent; the polyunsaturated glyceride content having been reduced by the "Kellogg Solexol Process" of propane solvent extraction. SAE 90 grade extreme pressure lubricant blends were prepared (1) using 18 percent of E.P. lubricant base, 1 percent dibenzyl disulfide as an additional extreme pressure agent and 81 percent of lubricating mineral oil and (2) using 9 percent of E.P. lubricant base, 1 percent of dibenzyl disulfide as an additional extreme pressure agent, and 90 percent of lubricating mineral oil. The solubility and viscosity index characteristics of extreme pressure lubricant blends containing the two different E.P. lubricant bases are shown in Table I, below.

Table I

| Blend No. | Fatty oil used in E.P. base                              | SAE 90 grade blend composition                                                                                                                                                                                     | 30-day storage stability                                                                                                      | V.I. |
|-----------|----------------------------------------------------------|--------------------------------------------------------------------------------------------------------------------------------------------------------------------------------------------------------------------|-------------------------------------------------------------------------------------------------------------------------------|------|
| 1.....    | Lard oil of 12 to 20% polyunsaturated glyceride content. | 18% wt. E.P. base.....<br>1% wt. dibenzyl disulfide.....<br>81% wt. Gulf Coast mineral oil (30 parts 160 Gulf Coast bright stock) (61 parts 200 Gulf Coast neutral).                                               | No separation of E.P. additive at room temp.<br>No separation of E.P. additive at 32° F.                                      | 89   |
| 2.....    | do.....                                                  | 18% wt. E.P. base.....<br>1% wt. dibenzyl disulfide.....<br>81% wt. Mid-Continent solvent refined mineral oil (36 parts 150 MCSR bright stock) (45 parts 170 MCSR neutral).                                        | Heavy separation of E.P. additive at room temp. within 48 hours. Heavy separation of E.P. additive at 32° F. within 48 hours. | 107  |
| 3.....    | Lard oil of 2% max. polyunsaturated glyceride content.   | 18% wt. E.P. base.....<br>1% wt. dibenzyl disulfide.....<br>81% wt. Mid-Continent solvent refined oil (37 parts 150 MCSR bright stock) (44 parts 170 MCSR neutral).                                                | No separation of E.P. additive at room temp.<br>No separation of E.P. additive at 32° F.                                      | 116  |
| 4.....    | Lard oil of 12 to 20% polyunsaturated glyceride content. | 9% wt. E.P. base.....<br>1% wt. dibenzyl disulfide.....<br>1.35% vis. index improver (Acrylid 150).....<br>88.65% mixed blend G.C. and MCSR oil (43 parts 160 Gulf Coast bright stock) (45.65 parts MCSR neutral). | do.....                                                                                                                       | 86   |
| 5.....    | do.....                                                  | 9% wt. E.P. base.....<br>1% wt. dibenzyl disulfide.....<br>90% wt. Mid-Continent solvent refined oil (50 parts 150 MCSR bright stock) (40 parts 170 MCSR neutral).                                                 | Heavy separation of E.P. additive at room temp.<br>Heavy separation of E.P. additive at 32° F.                                | 112  |
| 6.....    | Lard oil of 2% max. polyunsaturated glyceride content.   | 9% wt. E.P. base.....<br>1% wt. dibenzyl disulfide.....<br>90% wt. Mid-Continent solvent refined oil (51 parts 150 MCSR bright stock) (39 parts 170 MCSR neutral).                                                 | No separation of E.P. additive at room temp.<br>No separation of E.P. additive at 32° F.                                      | 110  |

mineral oils of the Pennsylvania and Mid-Continent solvent refined types.

It has been discovered that extreme pressure lubricant bases which are universally soluble in all types of lubricating mineral oils, including Pennsylvania, Mid-Continent solvent refined, Mid-Continent conventionally refined and Gulf Coastal mineral lubricating oils, can be prepared by employing a fatty material having a reduced polyunsaturated glyceride content in the preparation of the lubricant base. The polyunsaturated glyceride content of the fatty material is preferably reduced to a maximum of 6 percent for best results. Such reduction of polyunsaturated glyceride content of the fatty material can be brought about by treating the fatty material in accordance with the "Kellogg Solexol" process of propane solvent extraction or any other suitable method for the reduction of the polyunsaturated glyceride content of fatty materials.

The following example illustrates the advantages which are obtained by employing a material low in polyunsaturated glycerides as a fatty material in the preparation of sulfurized-phosphorized extreme pressure lubricant bases:

#### EXAMPLE I

Two extreme pressure lubricant bases were prepared in accordance with United States Patents 2,211,231 and 2,211,306, supra. One of the extreme pressure lubricant bases was prepared from lard oil having its normal polyunsaturated glyceride content, ranging from 12 to 20 per-

50 cent. The use of LPU lard oil as the fatty material in the preparation of extreme pressure lubricant additives can be further illustrated by the use of sulfurized LPU lard oil in cutting oil blends. Example II, below, describes the preparation of lubricants of this type.

#### EXAMPLE II

Cutting oil concentrates were prepared by heating a mixture of 9.71 percent of a fatty material and one-half of the total mineral oil component (43.58 percent) to a temperature of 280° to 300° F. When the desired temperature was obtained, 2.80 percent of sulfur was added slowly with stirring. The temperature was then raised to 320° to 330° F. and maintained at this level for 4 to 4½ hours. At the end of the reaction time, the sulfurized product was quenched with the remainder of the mineral oil (43.58 percent). The resulting cooled product was then stirred for one hour without additional heating and 0.03 percent of benzaldehyde was added as a deodorant. Table II, below, shows the characteristics of oil concentrates prepared in the manner described above using #1 lard oil of normal polyunsaturated glyceride content and LPU lard oil as the fatty materials and two different Mid-Continent mineral oils as the mineral oil component.

Table II

| Concen-<br>trate<br>No. | Fatty material                                       | Mineral oil                                                                                                   | Characteristics of finished blend |               |              |                       |              |                   |                                                                                                                                            |
|-------------------------|------------------------------------------------------|---------------------------------------------------------------------------------------------------------------|-----------------------------------|---------------|--------------|-----------------------|--------------|-------------------|--------------------------------------------------------------------------------------------------------------------------------------------|
|                         |                                                      |                                                                                                               | Grav-<br>ity<br>(API)             | Flash<br>° F. | Fire<br>° F. | Pour<br>point<br>° F. | Color<br>NPA | Percent<br>sulfur | Storage stability                                                                                                                          |
| 1.....                  | 9.71% #1 lard oil re-<br>acted with 2.80%<br>sulfur. | 87.49% solvent refined non-<br>viscous neutral.                                                               | 32.6                              | 405           | 460          | +20                   | Black        | 2.94              | Separation (phase and mar-<br>bling) at room temp. in 1<br>week. Heavy sulfur separa-<br>tion in 2 days at 32° F.                          |
| 2.....                  | 9.71% LPU lard oil<br>reacted with 2.80%<br>sulfur.  | do                                                                                                            | 32.6                              | 400           | 450          | +5                    | 8            | 2.77              | Slight trace peppery sediment<br>in 30 days at room temp.; in<br>30 days at 32° F. Minute<br>trace sulfur crystals in 5<br>weeks at 32° F. |
| 3.....                  | 9.71% #1 lard oil re-<br>acted with 2.80%<br>sulfur. | 48.12% non-viscous solvent re-<br>fined neutral. 39.37% sol-<br>vent extract from 100 vis-<br>cosity neutral. | 27.0                              | 375           | 430          | +10                   | -----        | 3.7               | Heavy sulfur and polymer<br>separation at room temp. and<br>at 32° F. in 1 month.                                                          |
| 4.....                  | 9.71% LPU lard oil<br>reacted with 2.80%<br>sulfur.  | do                                                                                                            | 27.0                              | 375           | 425          | +15                   | -----        | 3.63              | Slight polymer separation at<br>room temp. in 1 month. No<br>polymer separation at 32° F.<br>in 1 month.                                   |

It can be seen from Table II that the oil concentrates prepared from LPU lard oil were extremely stable in storage, while the concentrates prepared with lard oil of normal polyunsaturated glyceride content exhibited poor solubility characteristics as evidenced by their poor 45 stability in storage.

The solubility and viscosity index characteristics of sulfurized-phosphorized lubricant bases can also be improved by substituting 40 to 60 percent of wool grease for fatty materials having normal polyunsaturated glyceride content. In Example III, below, extreme pressure lubricant bases were prepared from a fatty material having normal polyunsaturated glyceride content and from mixtures of wool grease and a fatty material having normal polyunsaturated glyceride content.

### EXAMPLE III

Two extreme pressure lubricant bases were prepared according to the method disclosed in United States Patents 2,211,231 and 2,211,306, supra. One extreme pressure lubricant base was prepared from lard oil having its normal polyunsaturated glyceride content. A second extreme pressure lubricant base was prepared from a mixture of 50 percent wool grease and 50 percent of lard oil having its normal polyunsaturated glyceride content. SAE 90 grade extreme pressure lubricant blends were prepared using 9 percent of E.P. lubricant base, 1 percent of either dibenzyl disulfide or sulfurized terpene as the additional extreme pressure agent and 90 percent of lubricating mineral oil. The solubility characteristics of extreme pressure lubricant blends containing the two E.P. lubricant bases are shown in Table III, below.

it has been found that the high polyunsaturated glyceride content of fatty materials can be effectively modified by preparing sulfurized-phosphorized lubricant bases in a manner such that the viscosity of the finished extreme pressure lubricant base is below about 400 SUS at 210° F. The viscosity of the sulfurized-phosphorized extreme pressure lubricant base is preferably between about 150 and 400 SUS at 210° F. rather than above about 450 SUS at 210° F. as are the extreme pressure lubricant 50 bases heretofore used. The sulfurized and phosphorized extreme pressure lubricant bases having a viscosity below about 400 SUS at 210° F. can be prepared by carrying out the sulfurization and phosphorization at a temperature of about 300° to 350° F. while agitating with paddle-type agitators at a speed of about 15 to 50 revolutions per minute in an open or closed vessel. On the other hand, 25 the preparation of lubricant bases in accordance with methods heretofore considered most desirable requires aeration of the heated reaction mixture by dispersing air in the mixture either with or without agitation to obtain a product having a viscosity above about 400 SUS at 210° F. 30 The improvement in the solubility characteristics of extreme pressure lubricant bases attained by employing extreme pressure lubricant bases of low viscosity is illustrated by Example IV, below.

### EXAMPLE IV

Two sulfurized-phosphorized extreme pressure lubricant bases were prepared in accordance with United States Patents 2,211,231 and 2,211,306, supra, using lard oil having its normal polyunsaturated glyceride content 40 of 12 to 20 percent. One extreme pressure lubricant

Table III

| Blend<br>No. | Fatty oil used in E.P. base                                                      | SAE 90 grade blend composition                                                                                                                             | 90-day storage stability                                                                             |
|--------------|----------------------------------------------------------------------------------|------------------------------------------------------------------------------------------------------------------------------------------------------------|------------------------------------------------------------------------------------------------------|
| 1.....       | 50% wool grease.....<br>50% lard oil of 12 to 20% polyunsatu-<br>rate glyceride. | 9% E.P. base.....<br>1% dibenzyl disulfide.....<br>90% Mid-Continent solvent refined mineral oil<br>(63% 150 MCSR bright stock) (27% 170 MCSR<br>neutral). | Light separation of E.P. additive at room temp.<br>Trace separation of E.P. additive at 32° F.       |
| 2.....       | Lard oil of 12 to 20% polyunsatu-<br>rate glyceride content.                     | 9% E.P. base.....<br>1% dibenzyl disulfide.....<br>90% Mid-Continent solvent refined mineral oil<br>(61% 1120 MCSR oil) (29% 200 MCSR neutral).            | Heavy separation of E.P. additive at room temp.<br>Heavy separation of E.P. additive at 32° F.       |
| 3.....       | 50% wool grease.....<br>50% lard oil of 12 to 20% polyunsatu-<br>rate glyceride. | 9% E.P. base.....<br>1% sulfurized terpene.....<br>90% Mid-Continent solvent refined mineral oil<br>(55% 150 MCSR bright stock) (35% 170 MCSR<br>neutral). | Trace separation of E.P. additive at room temp.<br>Faint trace separation of E.P. additive at 32° F. |

It is to be observed that the lubricant blends containing wool grease-modified lard oil extreme pressure lubricant base were much more stable than the lubricant blend containing unmodified lard oil extreme pressure lubricant base.

Further, in accordance with the present invention, 75

base was prepared in a manner such that the viscosity of the finished base was 900 SUS at 210° F., while the other extreme pressure lubricant base was prepared in a manner such that the viscosity of the finished base was 276 SUS at 210° F. In this particular example the low viscosity extreme pressure lubricant base was prepared

by agitating the reaction mixture in an open kettle at a paddle speed of about 15 revolutions per minute and the high viscosity base was prepared by introducing finely dispersed air into the reaction mixture. Extreme pressure lubricant blends were prepared using 9 percent of the extreme pressure lubricant base, 1 percent of dibenzyl disulfide or sulfurized terpene as the additional extreme pressure agent and 90 percent of mineral oil. The storage stabilities of the extreme pressure lubricant blends thus prepared are set forth in Table IV.

higher while destearinized fatty materials of reduced high melting point saturate glyceride content will exhibit a pour point below +50° F. Example V illustrates the advantages obtained by preparing extreme pressure lubricant bases from fatty materials of reduced high melting point saturate glyceride content.

#### EXAMPLE V

In a series of tests, 6 extreme pressure lubricant bases 10 were prepared according to United States Patents 2,211,-

Table IV

| Blend No. | Description of E.P. base                                                           | SAE 90 grade blend composition                                                                                                                                                                                                                                                                                                                                                                                                                                            | 30-day storage stability                                                                                        |
|-----------|------------------------------------------------------------------------------------|---------------------------------------------------------------------------------------------------------------------------------------------------------------------------------------------------------------------------------------------------------------------------------------------------------------------------------------------------------------------------------------------------------------------------------------------------------------------------|-----------------------------------------------------------------------------------------------------------------|
| 1.....    | Sulfurized-phosphorized lard oil E.P. base having viscosity at 210° F. of 900 SUS. | 9% wt. E.P. base.....<br>1% wt. dibenzyl disulfide.....<br>90% wt. Mid-Continent solvent refined oil (61% 1120 MCSR oil) (29% 200 MCSR neutral).<br>9% wt. E.P. base.....<br>1% wt. sulfurized terpene.....<br>90% wt. Mid-Continent solvent refined oil (55% 120 MCSR bright stock) (32% 200 MCSR neutral).<br>18% wt. E.P. base.....<br>1% wt. sulfurized terpene.....<br>81% wt. Mid-Continent solvent refined oil (45% 120 MCSR bright stock) (36% 200 MCSR neutral). | Heavy separation of E.P. base after storage at room temp. Heavy separation of E.P. base after storage at 32° F. |
| 2.....    | Sulfurized-phosphorized lard oil E.P. base having viscosity at 210° F. of 276 SUS. | 1% wt. sulfurized terpene.....<br>90% wt. Mid-Continent solvent refined oil (55% 120 MCSR bright stock) (32% 200 MCSR neutral).<br>18% wt. E.P. base.....<br>1% wt. sulfurized terpene.....<br>81% wt. Mid-Continent solvent refined oil (45% 120 MCSR bright stock) (36% 200 MCSR neutral).                                                                                                                                                                              | No separation of E.P. base after storage at room temp. No separation of E.P. base after storage at 32° F.       |
| 3.....    | do.....                                                                            | 1% wt. sulfurized terpene.....<br>81% wt. Mid-Continent solvent refined oil (45% 120 MCSR bright stock) (36% 200 MCSR neutral).                                                                                                                                                                                                                                                                                                                                           | No separation of E.P. base after storage at room temp. No separation of E.P. base after storage at room temp.   |

Table IV effectively demonstrates that the extreme pressure lubricant blends containing the low viscosity extreme pressure lubricant base were highly stable and thus that this lubricant base was more compatible with high viscosity index mineral oil than was the high viscosity extreme pressure lubricant base.

It has also been found, in accordance with the present invention, that the low temperature characteristics of extreme pressure lubricant blends can be improved by employing sulfurized-phosphorized extreme pressure lubricant bases prepared from fatty materials of reduced high melting point saturate glyceride (also referred to as "stearin") content. The high melting point saturate glyceride content is also preferably reduced by treating the fatty material in accordance with the "Kellogg Solexol" process of propanesolvent extraction. A convenient measure of the high melting point saturate glyceride content is the pour point of the fatty material. For example, a fatty material of normal saturate glyceride content will exhibit a pour point of about +50° F. or

231 and 2,211,306, supra. Table V, below, sets forth 30 the characteristics of extreme pressure lubricant blends containing 18 percent of the extreme pressure lubricant base, 1 percent of sulfurized terpene as the additional extreme pressure agent and 81 percent of mineral oil. The extreme pressure lubricant bases used in lubricant blends 1a and 1b of Table V were prepared from LPU lard oil of normal saturate glyceride content and LPU lard oil of reduced high melting point saturate glyceride content, respectively. The extreme pressure lubricant bases of lubricant blends 2a and 2b were prepared from 35 wool grease-modified lard oil of normal saturate glyceride content and wool grease-modified lard oil of reduced high melting point saturate glyceride content, respectively. And lubricant blends 3a and 3b contained 40 extreme pressure lubricant bases of low viscosity prepared from lard oil of normal saturate glyceride content and lard oil of reduced high melting point saturate glyceride content, respectively.

Table V

| Blend No. | Fatty oil used in E.P. base                                                                                                                   | SAE 90 grade blend composition                                                                                                                                                                                                                                                                                                                                                                                                                                                                                                                                                                                                                                                                                                                                                                                                                                                                                                                                             | Pour point, °F. | 30-day storage stability                                         |
|-----------|-----------------------------------------------------------------------------------------------------------------------------------------------|----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----------------|------------------------------------------------------------------|
| 1a.....   | Lard oil of 1 to 2% polyunsaturate glyceride content and of ordinary "stearin" content and having a pour point of +50° F.                     | 18% wt. E.P. base.....<br>1% wt. sulfurized terpene.....<br>81% wt. Mid-Continent solvent refined oil (31% 120 MCSR bright stock) (50% 200 MCSR neutral).<br>18% wt. E.P. base.....<br>1% wt. sulfurized terpene.....<br>81% wt. Mid-Continent solvent refined oil (44% 120 MCSR bright stock) (37% 200 MCSR neutral).<br>18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (41% 150 MCSR Bright Stock) (40% 170 MCSR Neutral).<br>18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (40% 150 MCSR bright stock) (41% 170 MCSR neutral). | +20             | No separation of E.P. additive either at room temp. or at 32° F. |
| 1b.....   | Lard oil of 5 to 6% polyunsaturate glyceride content and destearinized to a pour point of +40° F.                                             | 18% wt. E.P. base.....<br>1% wt. sulfurized terpene.....<br>81% wt. Mid-Continent solvent refined oil (44% 120 MCSR bright stock) (37% 200 MCSR neutral).<br>18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (41% 150 MCSR Bright Stock) (40% 170 MCSR Neutral).<br>18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (40% 150 MCSR bright stock) (41% 170 MCSR neutral).                                                                                                                                                              | +10             | Do.                                                              |
| 2a.....   | 50% lard oil of 12 to 16% polyunsaturate glyceride content and ordinary "stearin" content and having a pour point of +50° F. 50% wool grease. | 18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (41% 150 MCSR Bright Stock) (40% 170 MCSR Neutral).<br>18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (40% 150 MCSR bright stock) (41% 170 MCSR neutral).                                                                                                                                                                                                                                                                                                                           | +35             |                                                                  |
| 2b.....   | 50% lard oil of 5 to 6% polyunsaturate glyceride content and destearinized to a pour point of +40° F. 50% wool grease.                        | 18% wt. E.P. base.....<br>1% wt. sulfurized terpene.....<br>81% wt. Mid-Continent solvent refined oil (41% 150 MCSR Bright Stock) (40% 170 MCSR Neutral).<br>18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (40% 150 MCSR bright stock) (41% 170 MCSR neutral).                                                                                                                                                                                                                                                                                                                                                                                                                                                                                        | +25             |                                                                  |
| 3a.....   | Lard oil of 12 to 16% polyunsaturate glyceride content and ordinary "stearin" content and having a pour point of +50° F.                      | 18% wt. E.P. base.....<br>1% wt. sulfurized terpene.....<br>81% wt. Mid-Continent solvent refined oil (44% 150 MCSR bright stock) (37% 170 MCSR neutral).<br>18% wt. E.P. base.....<br>1% wt. sulfurized terpene.....<br>81% wt. Mid-Continent solvent refined oil (40% 150 MCSR bright stock) (41% 170 MCSR neutral).                                                                                                                                                                                                                                                                                                                                                                                                                                                                                                                                                                                                                                                     | +25             |                                                                  |
| 3b.....   | Lard oil of 5 to 6% polyunsaturate glyceride content and destearinized to a pour point of +40° F.                                             | 18% wt. E.P. base.....<br>1% wt. sulfurized terpene.....<br>81% wt. Mid-Continent solvent refined oil (40% 150 MCSR bright stock) (41% 170 MCSR neutral).                                                                                                                                                                                                                                                                                                                                                                                                                                                                                                                                                                                                                                                                                                                                                                                                                  | +20             |                                                                  |

It is evident from the data of Table V that the lubricant blends containing extreme pressure lubricant bases prepared from fatty materials of reduced high melting point saturate glyceride content have superior low temperature characteristics when compared with lubricant blends containing extreme pressure lubricant bases prepared from fatty materials of normal saturate glyceride content.

The characteristics of the mineral oils employed in the specific examples set forth above are listed in Table VI, below. As has been pointed out above, the extreme pressure lubricant bases of this invention are universally soluble in mineral oils, and, therefore, mineral oils other than those employed in the specific examples can be utilized. It is generally conceded that solvent refined Mid-Continent mineral oils present the most severe problems relative to compatibility with additives, particularly extreme pressure lubricant additives. Thus, additives and bases which are soluble in Mid-Continent solvent refined mineral oils will also be soluble in other mineral oils.

Table VI  
TYPICAL TESTS FOR MINERAL OILS

| Mineral oil                                            | API gravity | COC flash | COC fire | SUS at 100° F. | SUS at 210° F. | Viscosity index | ° F. pour | Color, NPA | Percent sulfur |
|--------------------------------------------------------|-------------|-----------|----------|----------------|----------------|-----------------|-----------|------------|----------------|
| Solvent extract from 100 viscosity neutral             | 15.9        | 390       | 455      | 286            | 45.8           | 2               | +50       | +5         | 2.2            |
| Non-viscous neutral solvent refined Mid-Continent oil  | 36.6        | 370       | 405      | 71.3           | 36.7           | 111             | 0         | +1         | 0.18           |
| Gulf Coast oil                                         | 22.6        |           |          | 106            | 38.6           | 34              | -40       |            |                |
| 160 Gulf Coast bright stock                            | 17.8        | 515       | 590      | 6,530          | 151.6          | -15             | +30       | +3½        | 0.40           |
| 200 Gulf Coast neutral                                 | 22.8        | 355       | 390      | 207.3          | 43.5           | 21              | Below -30 | +3         |                |
| 150 Mid-Continent solvent refined bright stock         | 27.2        | 555       | 615      | 2,376          | 147            | 97              | +6        | +15        | 0.47           |
| 170 Mid-Continent solvent refined neutral              | 30.4        | 400       | 460      | 170.5          | 44.2           | 93              | +20       | +2         |                |
| 200 Mid-Continent conv. refined neutral                | 25.2        | 395       | 455      | 208.6          | 45.3           | 70              | +25       | +4         | 0.46           |
| Non-viscous Mid-Continent solvent refined neutral      | 36.6        | 370       | 405      | 71.3           | 36.7           | 111             | 0         | +1         | 0.18           |
| Extract from 100 Mid-Continent solvent refined neutral | 15.9        | 390       | 455      | 286            | 45.8           | 2               | +50       | +5         | 2.2            |
| 1120 Mid-Continent solvent refined oil                 | 24.8        |           |          | 1,623          | 118            | 98              | +15       |            |                |
| 200 Mid-Continent solvent refined neutral              | 29.7        | 410       | 470      | 201            | 46             | 91              | +10       | +1½        |                |
| 120 Mid-Continent solvent refined bright stock         | 25.8        | 540       | 600      | 1,985          | 125.5          | 91              | +15       | +7         |                |

The characteristics of the fatty materials employed in the specific examples of this specification are set forth in Table VII, below.

As has been indicated herein, suitable methods of sulfurizing or sulfuring and phosphorizing fatty materials are set forth in detail in United States Patents

Table VII  
TYPICAL TESTS FOR FATTY OILS

| Fatty material                                                               | Specific gravity | Flash, ° F. | Fire, ° F. | Pour point, ° F. | Saponification number | Iodine number | Titer, ° C. |
|------------------------------------------------------------------------------|------------------|-------------|------------|------------------|-----------------------|---------------|-------------|
| #1 lard oil                                                                  | 0.910-0.915      | 430-450     | 480-510    | 40-50            | 192-198               | 70-73         | 33-36.5     |
| LPU lard oil                                                                 |                  |             |            | 50               | 201                   | 69            |             |
| Lard oil of 1 to 2% polyunsaturated and of ordinary "stearin" content        |                  |             |            | +50              | 201                   | 69            |             |
| Lard oil of 5 to 6% polyunsaturated and destearinized to +40° F.             |                  |             |            | +40              | 200                   | 75            |             |
| Lard oil of 12 to 16% polyunsaturated content and ordinary "stearin" content |                  |             |            | +50              | 201                   | 74            |             |

Although lard oil has been employed as the fatty material in the specific examples contained herein, other fatty materials which contain substantial amounts of polyunsaturated glycerides and/or high melting point saturate glycerides can also be employed in the preparation of the extreme pressure lubricant additives and lubricants by following the teachings of the present invention. The term "fatty material" as employed in the specification and claims of this application is meant to include vegetable oils, animal fats and oils, and marine animal fats and oils. Typical examples of such fatty materials include sperm oil, hydrogenated soya oil, etc.

A suitable sulfurized terpene for use in the extreme pressure lubricant blends of this invention is the sulfurized terpene product prepared in accordance with United States Patent 2,443,823, issued to Lee Cone Holt on June 22, 1948. In addition to the sulfurized terpenes and dibenzyl disulfide set forth in the specific examples, other known extreme pressure agents may also be employed in the preparation of lubricant blends. Other deodorants than the benzaldehyde employed in Example II

60 2,211,231 and 2,211,306, supra. Briefly, sulfurized fatty materials may be prepared by heating the fatty material with sulfur or a compound of sulfur at a temperature below about 340° F. until the sulfur has reacted with the fatty material to form a product non-corrosive to a copper strip. Usually a reaction time of about 2 to 7 hours will be sufficient. A lubricant base containing chemically combined sulfur and phosphorous may be prepared by simultaneously sulfurizing and phosphorizing or by separately sulfurizing and then phosphorizing. In the former 65 case, both sulfurizing and phosphorizing agents are mixed with the fatty material being treated and the mixture is heated to a temperature below about 450° F. for from 2 to 8 hours, preferably at a temperature of 425° to 450° F. for 2½ hours. In the method whereby sulfurization and phosphorization are carried out in separate steps, a sulfurized fatty material, prepared in the manner outlined above, is mixed with a phosphorizing agent and the mixture is heated to a temperature below about 280° F. for a period from about 1 to 5 hours. As is more fully disclosed in United States Patent 2,211,306, supra, phos-

## 11

phorization is preferably carried out at a temperature of about 210° to 230° F. until the reagents have reacted sufficiently to prevent fuming of phosphorous when the temperature is raised above 230° F. (usually about 5 hours). After the product has reached a point at which phosphorous will not fume, the temperature may be raised to a temperature not exceeding about 350° F. to produce a highly stable product.

It is obvious from a consideration of the data presented herein and the accompanying discussion thereof that extreme pressure lubricant bases, which are universally soluble in mineral oils and which when added to suitable mineral oils produce extreme pressure lubricants of improved viscosity index and low temperature characteristics, can be prepared by sulfurizing or sulfurizing and phosphorizing a mixture of wool grease and a fatty material of low polyunsaturated glyceride and high melting point glycerol ester content under conditions such that a product having a viscosity below about 400 SUS at 210° F. is obtained.

Having described and illustrated the nature of this invention, what is claimed is:

1. The preparation of an extreme pressure lubricant additive having improved storage stability and low tem-

perature characteristics when blended with solvent refined mineral lubricating oil from natural fatty material having a content of polyunsaturated glycerol esters of high boiling fatty acids exceeding about 10%, which esters when chemically reacted with sulfur and phosphorus tend to form sulfur and phosphorus-containing reaction products insoluble in said lubricating oil, comprising reducing the content of said polyunsaturated glycerol esters to about 1.0 to 2.0 weight percent, then sulfurizing and phosphorizing said material during mechanical agitation without blowing with an oxidizing medium under conditions of time and temperature such that a product having a viscosity below about 400 SUS at 210° F. is produced.

2. The method in accordance with claim 1 in which said natural fatty material is lard oil and the pour point of said lard oil is below about 50° F. prior to said reactions.

## References Cited in the file of this patent

## UNITED STATES PATENTS

|           |                      |               |
|-----------|----------------------|---------------|
| 2,483,600 | Stucker et al. ----- | Oct. 4, 1949  |
| 2,542,161 | Stucker -----        | Feb. 20, 1951 |
| 2,678,937 | Brennan et al. ----- | May 18, 1954  |